

S. O. COWPER-COLES.  
SCALING AND ANNEALING METALS.  
APPLICATION FILED OCT. 10, 1911.

1,047,616.

Patented Dec. 17, 1912.



Witnesses.

J. R. Moore  
R. L. S. Barry.

Inventor.

Sherard Osborne Cowper-Coles  
By Whitelaw Reed, Atty.

# UNITED STATES PATENT OFFICE.

SHERARD OSBORN COWPER-COLES, OF WESTMINSTER, LONDON, ENGLAND.

## SCALING AND ANNEALING METALS.

1,047,616.

Specification of Letters Patent. Patented Dec. 17, 1912.

Application filed October 10, 1911. Serial No. 653,825.

To all whom it may concern:

Be it known that I, SHERARD OSBORN COWPER-COLES, a subject of the King of Great Britain, residing at 82 Victoria street, 5 Westminster, London, England, have invented new and useful Improvements in Scaling and Annealing Metals, of which the following is a specification.

My invention relates to improvements in 10 the existing methods of scaling and annealing metals, which metals may be subsequently coated with other metals, enamels, lacquers or the like, if desired, and to that class of process described in the specification of former Letters Patent No. 979,931 (dated December 27, 1910), wherein metallic articles to be scaled and annealed are heated in an atmosphere of a reducing gas.

In carrying out such a process as that described in the specification of the aforesaid patent, it is found advantageous to cool the articles rapidly owing to the fact that if the articles are cooled slowly a deleterious film is deposited on the surface of the clean 25 metal.

As the result of experiment I have discovered that, if, during the scaling and annealing operation the metallic articles are inclosed in an envelop that the film hereinbefore referred to is not formed, and my invention, therefore, consists in inclosing the articles to be treated in a vessel or envelop which may entirely inclose the articles, so that the reducing gases will have to penetrate the substance of the said vessel or envelop, or may have formed in it openings, which, while allowing contact of the reducing gases with the metallic articles, for effecting the reduction of the scale, do not 35 allow access of the deleterious gases to the said articles on account of the slow diffusion of such gases when cooling down.

The envelop in which the articles are inclosed may be of cast or wrought iron, or 45 of unglazed earthenware, or any other material through which the reducing gases will diffuse at or about the annealing temperature.

It will be understood that when the envelop is formed of metal, as for example, wrought iron, the reducing gases diffuse through the said envelop when the latter is at a high temperature in a sufficient quantity to reduce the scale and oxid upon the 55 articles within the envelop to the metallic state. When the envelop containing the ar-

ticles, however, is withdrawn into the cooling chamber the deleterious gases do not diffuse through the envelop, and when the latter is open are found to penetrate through 60 the openings only for a relatively short distance, so that by making the envelop of the proper dimensions all the articles contained therein can be kept out of contact with these gases.

My invention will be readily understood by reference to the accompanying drawing, in which:

Figure 1 is a longitudinal section illustrating a vessel or envelop made of two 70 metal plates which are united at the edges, and which are represented as inclosing between them a series of metal plates to be scaled. Fig. 2 is a sectional elevation of a vessel which may be made of cast iron or of 75 unglazed earthenware and which is represented as being in two parts, the lower part being formed with a channel into which the edge of the other part is inserted and sealed by means of sand or other suitable material 80 which forms a porous joint through which only the reducing gases will penetrate. Fig. 3 is a transverse section on the line 3—3, Fig. 2. Fig. 4 is a view somewhat similar to Fig. 1, except that the edges of the plates at 85 the ends of the envelops are represented as being arranged at a short distance apart, so as to leave a restricted opening, it being found in practice, that, owing to the very slow diffusion of the deleterious gases contained 90 in the reducing gases, these deleterious gases do not penetrate the restricted openings to any appreciable extent, while the articles are cooling down. It is found, for example, in practice, that the distance to which the 95 deleterious gases penetrate through the openings, is roughly four times the smaller dimension of any particular opening; for instance, if the opening be 6 inches by 1 inch 100 in cross section, the distance the deleterious gases would penetrate into the envelop would be 4 inches, this being four times the smaller dimension of the opening. It results that if the distance the articles are placed from any particular opening exceeds 105 four times the smaller dimension of such opening the deleterious gases will not travel into the envelop sufficiently far to reach the articles.

The articles inclosed in a vessel or envelop such as above described are introduced into the scaling and annealing chamber and

heated therein to the required temperature, until the whole of the metallic oxide on the surface of the metallic articles is reduced to a metallic state by the reducing gases which penetrate into the vessel either through the walls thereof, or through the restricted openings which are left, as in the case of the arrangement shown in Fig. 4 or, as in the arrangement shown in Figs. 2 10 and 3.

The scaling operation having been completed the vessel is withdrawn into the cooling chamber, as described in the specification before referred to, and remains there 15 until the temperature falls to about 150° C., the envelop preventing the articles from coming into contact with any gases which would produce the film before referred to.

Claims.

- 20 1. A process for removing scale from and annealing metals which consists in inclosing the articles to be treated, in an envelop placing the articles and envelop in the annealing chamber and heating it in an atmosphere of reducing gas which penetrates the substance of the walls of the envelop, for the purpose of scaling the metallic contents thereof, and in then allowing the envelop and its contents to cool in a reducing gas 25 for the purpose of annealing the contents, the deleterious gases during the cooling

process being maintained out of contact with the metallic articles by the walls of the inclosing envelop.

2. The process of removing scale from 35 metals, which consists in inclosing the articles to be treated in an envelop, placing said articles and envelop in an annealing chamber, supplying said chamber with reducing gas and heating said chamber, the said envelop permitting said reducing gas to pass into the interior of the same into contact with said articles, and preventing the contact of deleterious gases therewith. 40

3. The process of removing scale from 45 metals and annealing the same, which consists in inclosing the articles to be treated in an envelop, placing the articles and envelop in an annealing chamber, supplying reducing gas to said chamber and heating 50 said chamber, and then allowing said envelop and its contents to cool in the same conditions, the said envelop permitting the reducing gas to pass into the interior of the same and into contact with said articles and 55 preventing the contact of deleterious gases therewith.

SHERARD OSBORN COWPER-COLES.

Witnesses:

JOHN E. BOUSFIELD,  
E. E. DABBS.